

Feb. 16, 1926.

1,572,975

J. W. VAN METER  
METHOD OF HEATING METAL, GLASS, OR OTHER  
MATERIAL TO RENDER THE SAME WORKABLE  
Filed June 5, 1922



James W. Van Meter  
By J. C. Garner  
Attorney

## UNITED STATES PATENT OFFICE.

JAMES W. VAN METER, OF SAN RAFAEL, CALIFORNIA.

## METHOD OF HEATING METAL, GLASS, OR OTHER MATERIAL TO RENDER THE SAME WORKABLE.

Application filed June 5, 1922. Serial No. 566,204.

*To all whom it may concern:*

Be it known that I, JAMES W. VAN METER, a citizen of the United States, and resident of San Rafael, Marin County, State of California, have invented a new and useful Method of Heating Metal, Glass, or Other Material to Render the Same Workable, of which the following is a specification.

This invention relates to improvements in methods of heating metal, glass or other material to render the same workable, the object of the invention being to provide an improved method by which such material can be heated in a very short time, at minimum cost, and without the employment of expensive furnaces or apparatus, and without the employment of fire or electric current, and which is effective to render such material and any article made thereof, when so treated, sufficiently hot to enable the same to be bent, shaped, cut, or rendered otherwise workable, the invention consisting in exposing such material to the action of heat generated by the chemical reaction of a reaction causing agent, such as for instance, chlorine, on a body of initially inert material such as for instance, particles of zinc, iron, lead, arsenic, or other metal, as hereinafter described and claimed.

30 In the accompanying drawing:—

Fig. 1 is a diagram, partly in elevation and partly in section, showing a pipe in an initial stage of treatment in accordance with my improved method, preparatory to bending.

35 Fig. 2 is a similar view, showing the pipe bent.

Fig. 3 is a similar view showing a body of material such as metal or glass in the act of being heated from the exterior in accordance with my improved method.

In accordance with my improved method, for the purpose of heating an article made of metal, glass or other material for the purpose of rendering the same workable, I provide a sufficient charge or body of material which is initially inert and which may consist preferably of sawdust, which contains some moisture, bran, or the like, and mix the same intimately with an initial-

ly inert material, such for instance, particles of zinc, iron, lead, or other metal, or arsenic. Such a charge is indicated diagrammatically at 1, and assuming that the work is a tube 2 of iron, glass or other material, and 55 it is required to heat the same, interiorly, to render the same workable so that it can be bent or fashioned as may be desired, I confine the said body or charge of initially inert material in the said tube, at the required or desired point by means of wads 3 which are preferably made of loose asbestos or other material which is readily permeable by gas and air.

I also provide a sufficient quantity of a 65 reaction causing agent, such as for instance, chlorine, which is here diagrammatically shown as contained under pressure in a liquid state in a tank 4. Said tank has a valve 5 which may be opened or closed at 70 will to control the passage of chlorine gas from the tank to the work or pipe through a tube 6 which is here shown as entering one end of the pipe or other work 2 through a suitable stopper 7. I also preferably provide means to force air through the said tube to the charge or body of initially inert material in the work and for the purpose of this specification I show a container 8 for compressed air, which container is provided 80 with a suitable controlling valve 9, and communicates with the tube 6 through a tube 10. An escape tube 11 is also in most instances desirable in order to protect the operative from the fumes, and is here shown 85 as leading through a stopper 12 in the work pipe, and may be carried and arranged to discharge into the outer air or into a vessel of water or other place where the fumes may be absorbed or neutralized. In order to enable any desired pressure to be attained in the work tube during the chemical reaction of the chlorine on the metallic particles, I also provide the escape tube 11 with a valve 11<sup>a</sup>, which may be opened or closed 90 to any desired extent or at any time required.

In order then to heat the work and render the same workable, it is only necessary to open the valve of the chlorine tank and 100

thus permit chlorine to enter the work 2 and to pass through the charge of initially inert material therein, through the asbestos wads. As the chlorine comes in contact 5 with the initially inert material constituting the body of the charge it reacts chemically on the metal particles, zinc, iron, lead or the like in the charge, and as the result of such chemical reaction an intense heat is 10 instantaneously developed, without the aid of oxygen, and to which the work is exposed, and by which the work, whether as in this instance a pipe, or other article or object, and whether made of iron, steel, or 15 other metal, or of glass, porcelain or other material, is in a very short space of time rendered workable so that it can be bent as shown in Fig. 2, or otherwise worked as may be desired.

20 The sawdust or other moisture containing material in the charge of initially inert material forms a core when the method is being carried out in the interior of a hollow object such as a pipe, as here shown, and 25 is ignited by the heat generated by the chemical reaction of the chlorine on the metallic particles, and caused to burn, but not to be completely consumed, and hence remains as in the form of charcoal in the work pipe 30 or other hollow object and forms a filler therein which prevents the pipe or other hollow object from being distorted cross sectionally while being bent. A binding material, such as a hydrocarbon oil, may be 35 used advantageously in some instances in forming the body or core and it also acts to retain the moisture in the sawdust particles.

40 The bending may be done manually if the pipe or other work object is of ordinary size, or may be bent or otherwise worked by any suitable mechanical or other means, within the scope of my invention.

45 The compressed air is only used for forcing all of the fumes from the work tube and out of the vicinity, and for scavenging and cooling the work.

50 An especial advantage results from the use of my method in heating a pipe to render the same bendable, as by means of my method the pipe can be heated from the inside.

55 My improved method can also with equal facility be employed in heating an object from the outside in order to render the same workable and in Fig. 3 I illustrate diagrammatically how this can be done, the work 11<sup>b</sup> being embedded in a charge 12<sup>a</sup> of the initially inert material, in a suitable receptacle such as for instance an oven or furnace 13, and the chlorine being introduced through a pipe 14 and the gases emitted through a flue 15.

60 For bending a two-inch iron tube, such 65 for instance as a boiler tube, I have ordi-

narily used about two pounds of material in about the following proportions: metal particles 1½ pounds, sawdust ½ pound, chlorine (liquid) about ¼ pound. These proportions may be varied according to the thickness of the tube, and as a general rule enough of the material should be used to fill that portion of the tube which is to be bent or otherwise worked. For working material such as glass, a smaller quantity 75 of the material may be employed.

I would have it understood that the term "workable" as used in the foregoing description and in the appended claims is to be construed as covering the annealing of material by my improved heating process as well as the bending, shaping, forming or otherwise performing work of any kind on such material.

75 What I claim is:—

1. The herein described method of heating metal, glass and other materials to render the same workable, consisting in exposing such material to the action of heat generated in a non-oxidizing atmosphere by the 90 chemical reaction of a reaction causing agent on a body of initially inert material.

2. The herein described method of heating metal, glass and other material, to render the same workable, consisting in exposing such material to the action of heat generated by the chemical reaction of a reaction causing agent, on a body of initially inert material.

3. The method of rendering metal, glass and other material workable, consisting in exposing the same to the action of heat generated in a non-oxidizing atmosphere by the chemical reaction of a reaction causing agent on initially inert material.

4. The method of rendering metal, glass and other material workable, consisting in exposing the same to the action of heat generated in a non-oxidizing atmosphere by the chemical reaction of a reaction causing agent on metallic particles.

5. The method of rendering metal, glass or other material workable, consisting in associating the same with a charge or body of initially inert material and causing such initially inert material to be acted upon by a reaction causing agent, to generate heat in a non-oxidizing atmosphere which is communicated to such metal or other material.

6. The method of rendering a hollow object of metal, glass or other material workable, consisting in placing in such hollow object a charge or body of initially inert material and introducing to such charge or body of initially inert material a reaction causing agent, to generate heat in a non-oxidizing atmosphere.

7. The method of rendering a hollow object of metal, glass or other material workable, consisting in placing in such hollow

object a core of combustible material containing moisture, together with initially inert material and subjecting such core to the action of a reaction causing agent to generate heat in a non-oxidizing atmosphere.

8. The method of rendering metal, glass and other material workable, consisting in

exposing the same to the action of heat generated in a non-oxidizing atmosphere by the chemical reaction of a reaction causing agent <sup>10</sup> under pressure, on initially inert material.

In witness whereof I affix my signature.

JAMES W. VAN METER.